

## UNITED STATES PATENT OFFICE

1,989,100

PROCESS FOR IMPROVING ARTIFICIAL  
FIBROUS MATERIAL

Leon Lilienfeld, Vienna, Austria

No. Drawing. Application May 29, 1929, Serial  
No. 367,154. In Austria June 16, 1928

11 Claims. (Cl. 8—20)

This invention is based on my discovery that artificial fibrous materials, for example, artificial silk, are in many respects improved in respect of their properties, by treating them with one or more substances having a basic reaction, at a high or moderately raised temperature. The most important basic substances for the purpose of this invention are solutions of caustic alkalies or of alkali metal sulphides.

10 The improvements which are attained by the treatment of the artificial fibre (such as artificial silk) in accordance with this invention may be summarized as follows:—

15 (1) The material acquires a soft, full, elastic feel approaching, and in some cases, equaling that of natural silk;

20 (2) The undesirable metallic lustre of the material is modified to give a pleasing and more natural lustre and appearance, and may approach and in some cases equal the lustre of natural silk.

25 (3) The elasticity and extensibility of the material are increased.

30 (4) The undesirable tendency of the material, in contrast with natural silk, to become creased, that is to say, in wearing, creases (particularly in the case of fabrics) which do not disappear by themselves, is very much diminished and in some cases altogether eliminated.

35 (5) The known difficulties experienced in mercerizing the cotton content of mixed fabrics or of other mixed textiles consisting of cotton and artificial silk are eliminated by using alkali solutions or alkali metal sulphide solutions at a raised temperature for the mercerization of such materials; hitherto these difficulties could be minimized only by artificial aids, such as a pre-treatment of the artificial threads or fibers with a protective sizing or by the use of special mercerizing solutions, containing an agent for preventing great injury to the artificial silk.

40 The invention has appreciable advantages in its application to the treatment of staple fibre and artificial wool; also these advantages reside essentially in an improvement in the feel of the material, in an increase in the elasticity and in a diminution in the tendency of the material to acquire permanent creases.

45 My investigations have, in fact, shown that the process of the invention is well suited for modifying artificial silk so that it closely resembles natural silk in many of its properties.

50 Finally, it may be mentioned that it is indicated by my investigations that artificial silk which has been treated in accordance with this invention, has lost wholly or in considerable degree its tendency towards irregular absorption of dyestuffs.

55 The observation on which the invention is based, that the elasticity and feel of artificial

fibrous material is appreciably improved by treatment with a hot solution of a caustic alkali or of an alkali metal sulphide of suitable concentration, without being considerably affected in respect of its strength in the wet and in the dry state and without destruction of its lustre, the latter being in many cases improved, is surprising in view of the knowledge that solutions of caustic alkalies of the same concentration, (particularly from about 5 to about 40 per cent. 10 strength, calculated as NaOH) when used at ordinary temperatures, but otherwise under the same conditions have no effect or no appreciable effect on the elasticity of artificial silk and generally reduce its lustre and decrease its strength 15 by an appreciable amount.

20 The invention consists in a treatment of artificial fibrous material (including pure and mixed fibres and fabrics, as hereinafter explained) with a solution of a basic substance, particularly a solution of a caustic alkali or of an alkali sulphide, at a high temperature, for example at 50–120° C. or higher, or at a moderately raised temperature, for example at 25–50° C.

25 The invention may be applied to viscose silk 25 of any kind including the particular type of viscose silk (hereinafter referred to as Lilienfeld silk) made by spinning viscose in a bath containing a strong mineral acid, particularly strong sulphuric acid (as described for example in U. S. 30 Patents Nos. 1,683,199 and 1,683,200). It may also be applied to cuprammonium and silk, to nitro-silk (the above mentioned silks being composed essentially of cellulose or cellulose hydrate and are hereinafter included in the terms "artificial fibrous material of regenerated cellulose" 35 and "regenerated cellulose artificial silk", for brevity) and when there is used a strong solution of a caustic alkali (such as a solution containing more than about 30 per cent. of caustic alkali, calculated as NaOH) or a strong solution of an alkali metal sulphide (such as a solution containing from 84 to 100 per cent. of sodium sulphide, calculated as the crystalline material, Na<sub>2</sub>S·9H<sub>2</sub>O) to acetate silk.

40 The invention is applicable not only to artificial fibres as such (for example artificial silk, staple fibre, artificial wool, artificial hair, artificial straw) in the form of spun material (threads, yarns in skeins or cops, or in the form 45 of warps, twisted yarn or the like) but also to artificial fibres in the form of a fabric. It is furthermore applicable both to threads and fabrics consisting wholly of artificial fibres, and to mixed threads and fabrics, that is to say, to threads and fabrics containing in addition to artificial fibres another fibrous material or materials, such as a mercerizable fibre like cotton, or another fibre, such as natural silk, sheep's wool or the like. If wool or real silk is present 50

55 60

they have to be protected against the action of the hot or warm solution of alkali by a suitable impregnation. The expression "artificial fibrous material" as used in this specification and 5 claims is intended to include artificial fibres (prepared from viscose, cuprammonium cellulose solution, nitrocellulose solution, cellulose acetate solution). The fibres may be artificial silk, artificial cotton, artificial wool, artificial hair or 10 artificial straw, these being in the form of spun material (threads, yarns in skeins or cops, or in the form of warps, twisted yarn or the like or in the form of fabrics) consisting of, or containing 15 such spun materials. It includes ordinary viscose silk as well as "Lilienfeld silk".

Among the basic substances which find application in the invention, solutions of caustic alkalies and of alkali metal sulphides have been found especially advantageous; in the case of 20 alkali metal sulphides, however, the concentration of the solution should not be less than 15 per cent., the sulphide being calculated as crystalline sodium sulphide. Solutions of other basic substances, however, may be used, such as 25 quaternary ammonium bases, organic bases (for example, guanidine) in whose aqueous solutions there may be presumed to be present a hydroxide which is strongly electrolytically dissociated or sulphonium hydroxides, such as trimethylsulphonium hydroxide. 30

The basic substance may be used in conjunction with a salt having a neutral or alkaline reaction (such as sodium chloride, sodium sulphate, sodium silicate, sodium aluminate, sodium 35 zincate, borax, a sodium phosphate, sodium

acetate), or with a monohydric or polyhydric alcohol, such as ethyl alcohol or glycerin, a suitable quantity of the salt or alcohol being incorporated in the solution of the basic substance.

The invention may be applied to finished artificial fibrous material initially, in the dry state, or in the wet or moist state; it may also be applied to artificial fibrous material which is not completely finished, for example, before or after the washing operation which succeeds the spinning of the fibre.

In cases in which a high elasticity is required of the treated material, the treatment is applied without subjecting the material to tension, or whilst subjecting it only to moderate tension.

The following Tables I and II illustrate how the invention may be carried out, and show the results obtained by treating artificial fibrous materials in accordance with the invention and, for comparison, the results obtained by a treatment conducted at ordinary temperature but under otherwise identical conditions:—

Table I

In the Examples 1-20 described in the following table, ordinary viscose silk (titre: 150 deniers in 24 single filaments; strength in the dry state: 1.676 grams per denier; strength in the wet state: 0.600 grams per denier; extensibility: 24.2 per cent; elasticity: 8.2 per cent) was treated by immersion in the shrinking agents indicated in column 1 in the form of skeins without application of tension, at the temperature indicated in column 2 for the period indicated in column 3. 35

| Ex-<br>ample | Shrinking<br>agent | Tem-<br>pera-<br>ture      | Duration<br>of action | After-treatment                                                                                                                                    | Lustre                                                                | Feel                                     | Titre      | Strength per<br>denier |                 | Extens-<br>ibility | Elast-<br>icity | 40           |    |
|--------------|--------------------|----------------------------|-----------------------|----------------------------------------------------------------------------------------------------------------------------------------------------|-----------------------------------------------------------------------|------------------------------------------|------------|------------------------|-----------------|--------------------|-----------------|--------------|----|
|              |                    |                            |                       |                                                                                                                                                    |                                                                       |                                          |            | In dry<br>state        | In wet<br>state |                    |                 |              |    |
| 45           | 7% NaOH            | Degrees<br>centi-<br>grade | 15                    | 1 minute...                                                                                                                                        | 1 minute in boiling<br>water, washed<br>with cold water<br>and dried. | Considerably<br>destroyed.               | Stiff..... | Deniers<br>165         | Grams<br>1.139  | Grams<br>.348      | Percent<br>17   | Percent<br>5 | 45 |
|              |                    |                            |                       |                                                                                                                                                    |                                                                       |                                          |            |                        |                 |                    |                 |              |    |
|              |                    |                            |                       |                                                                                                                                                    |                                                                       |                                          |            |                        |                 |                    |                 |              |    |
| 50           | 2.....do.....      | 25                         | do.....               | do.....                                                                                                                                            | High.....                                                             | Soft.....                                | 168        | 1.348                  | .476            | 34                 | 10              | 7            |    |
|              | 3.....do.....      | 15                         | do.....               | 5 minutes in sul-<br>phuric acid of<br>10 per cent.<br>strength at 15°<br>C., 1 minute in<br>boiling water,<br>washed with cold<br>water and dried | Considerably<br>destroyed.                                            | Stiff.....                               | 168        | 1.303                  | .414            | 21                 |                 |              |    |
| 55           | 4.....do.....      | 25                         | do.....               | do.....                                                                                                                                            | High.....                                                             | Soft.....                                | 164        | 1.411                  | .475            | 31                 | 10              | 7.8          |    |
|              | 5.....10% NaOH     | 15                         | do.....               | 5 minutes in sul-<br>phuric acid of<br>10 per cent.<br>strength at 15°<br>C., finally<br>washed and<br>dried                                       | Destroyed.....                                                        | Wiry.....                                | 192        | 0.697                  | .279            | 57.8               |                 | 55           |    |
| 60           | 6.....do.....      | 100                        | do.....               | do.....                                                                                                                                            | Completely<br>retained and<br>improved.                               | Extraordi-<br>narily soft and<br>elastic | 164        | 1.442                  | .472            | 27.8               | 9.2             | 60           |    |
|              | 7.....12% NaOH     | 15                         | do.....               | do.....                                                                                                                                            | Practically<br>destroyed                                              | Opaque                                   | 180        | 0.851                  | .316            | 41.4               | 4.8             |              |    |
| 65           | 8.....do.....      | 100                        | do.....               | do.....                                                                                                                                            | Completely<br>retained and<br>improved.                               | Soft and elas-<br>tic                    | 164        | 1.463                  | .478            | 28.2               | 11.6            |              |    |
|              | 9.....15% NaOH     | 15                         | do.....               | do.....                                                                                                                                            | Very much<br>diminished                                               | Soft.....                                | 184        | 1.001                  | .343            | 42.4               | 7.8             | 65           |    |
| 70           | 10.....do.....     | 100                        | do.....               | do.....                                                                                                                                            | Completely<br>retained and<br>improved.                               | Soft and elas-<br>tic                    | 164        | 1.274                  | .446            | 30.6               | 13.3            |              |    |
|              | 11.....18% NaOH    | 15                         | do.....               | do.....                                                                                                                                            | Very much di-<br>minished.                                            | Somewhat soft                            | 184        | 1.115                  | .389            | 39.7               | 8.4             | 70           |    |
| 75           | 12.....do.....     | 100                        | do.....               | do.....                                                                                                                                            | Completely<br>retained and<br>improved.                               | Soft and elas-<br>tic.                   | 164        | 1.350                  | .469            | 31.4               | 12.1            |              |    |
|              | 13.....20% NaOH    | 15                         | do.....               | do.....                                                                                                                                            | Very much di-<br>minished.                                            | Slightly stiff-<br>ened.                 | 174        | 1.173                  | .392            | 37.1               | 6.8             |              |    |
|              | 14.....do.....     | 100                        | do.....               | do.....                                                                                                                                            | Completely<br>retained and<br>improved.                               | Soft and elas-<br>tic.                   | 166        | 1.355                  | .516            | 32                 | 16              |              |    |

| Ex-<br>ample | Shrinking<br>agent      | Tem-<br>pera-<br>ture      | Duration<br>of action | After-treatment | Lustre                                                                                                   | Feel                                    | Titre                  | Strength per<br>denier |                 | Extens-<br>ibility | Ela-<br>sticity      |                     |
|--------------|-------------------------|----------------------------|-----------------------|-----------------|----------------------------------------------------------------------------------------------------------|-----------------------------------------|------------------------|------------------------|-----------------|--------------------|----------------------|---------------------|
|              |                         |                            |                       |                 |                                                                                                          |                                         |                        | In dry<br>state        | In wet<br>state |                    |                      |                     |
| 5            |                         |                            |                       |                 |                                                                                                          |                                         |                        |                        |                 |                    | 5                    |                     |
| 15           | 22½%<br>NaOH.           | Degrees<br>centi-<br>grade | 15                    | 1 minute...     | 5 minutes in sul-<br>phuric acid of 10<br>percent strength<br>at 15° C., finally<br>washed and<br>dried. | Very much di-<br>minished.              | Stiff.....             | Deniers<br>178         | Grams<br>1.165  | Grams<br>.400      | Per-<br>cent<br>40.5 | Per-<br>cent<br>7.2 |
| 10           |                         |                            |                       |                 |                                                                                                          |                                         |                        |                        |                 |                    | 10                   |                     |
| 16           | do                      | 120                        | do                    | do              | do                                                                                                       | Completely<br>retained and<br>improved. | Soft and elas-<br>tic. | 166                    | 1.394           | .462               | 30.1                 | 11.5                |
| 15           | 50% NaOH.               | 100                        | do                    | do              | do                                                                                                       | do                                      | do                     | 158                    | 1.492           | .553               | 26.8                 | 7.5                 |
| 18           | 75% NaOH.               | 150                        | do                    | do              | do                                                                                                       | do                                      | do                     | 160                    | 1.537           | .443               | 27.4                 | 10.1                |
| 19           | 84% Na <sub>2</sub> S.  | 100                        | 5 minutes             | do              | do                                                                                                       | do                                      | do                     | 155                    | 1.551           | .588               | 30.3                 | 9.7                 |
| 20           | 100% Na <sub>2</sub> S. | 100                        | do                    | do              | do                                                                                                       | do                                      | do                     | 162                    | 1.506           | .563               | 33.5                 | 13.5                |

Table II

In the following table, the treatment was as indicated at the head of Table I, but the parent material was a number of samples of "Lilienfeld-silk", that is viscose silk made by spinning vis-  
cose in a sulphuric acid bath of 55° Bé, according to the process set forth in my U. S. Patents 1,683,199 and 1,683,200, above mentioned. For a further comparison are added the physical constants of the untreated material.

20 25 20 25

| Ex-<br>ample | Shrinking<br>agent       | Tem-<br>pera-<br>ture      | Duration<br>of action | After-treatment                                                                                                                                        | Lustre                                                                | Feel                                                         | Titre                   | Strength per<br>denier |                         | Extens-<br>ibility      | Ela-<br>sticity             |                            |
|--------------|--------------------------|----------------------------|-----------------------|--------------------------------------------------------------------------------------------------------------------------------------------------------|-----------------------------------------------------------------------|--------------------------------------------------------------|-------------------------|------------------------|-------------------------|-------------------------|-----------------------------|----------------------------|
|              |                          |                            |                       |                                                                                                                                                        |                                                                       |                                                              |                         | In dry<br>state        | In wet<br>state         |                         |                             |                            |
| 30           |                          |                            |                       |                                                                                                                                                        |                                                                       |                                                              |                         |                        |                         |                         | 30                          |                            |
| 35           | 21 Untreated<br>7% NaOH. | Degrees<br>centi-<br>grade | 15                    | 1 minute...                                                                                                                                            | 1 minute in boiling<br>water, washed<br>with cold water<br>and dried. | Destroyed.....                                               | Stiff, hard,<br>coarse. | Deniers<br>74          | Grams<br>5.527<br>2.618 | Grams<br>3.770<br>0.900 | Per-<br>cent<br>6.5<br>10.2 | Per-<br>cent<br>4.5<br>6.2 |
| 40           | 22 Untreated<br>7% NaOH. | 25                         | 1 minute...           | 1 minute in boiling<br>water, washed<br>with cold water<br>and dried.                                                                                  | Retained.....                                                         | Soft.....                                                    | 42                      | 4.654<br>50            | 2.988<br>2.480          | 6.2<br>12.7             | 4.2<br>6.1                  |                            |
| 45           | 23 Untreated<br>7% NaOH. | 15                         | 1 minute...           | Washed with cold<br>water and dried.                                                                                                                   | Destroyed.....                                                        | Stiff, coarse<br>filaments<br>pasted to-<br>gether.          | 63                      | 5.730<br>83            | 4.365<br>3.042          | 5.3<br>9                | 4<br>5.7                    |                            |
| 50           | 24 Untreated<br>7% NaOH. | 25                         | 1 minute...           | Washed with cold<br>water and dried.                                                                                                                   | Retained.....                                                         | Soft.....                                                    | 80                      | 6.108<br>75            | 4.701<br>5.500          | 5.7<br>11               | 4.4<br>6.4                  |                            |
| 55           | 25 Untreated<br>7% NaOH. | 15                         | 1 minute...           | 5 minutes in sul-<br>phuric acid of<br>10 per cent.<br>strength at 15°<br>C., washed with<br>cold water and<br>dried.                                  | Destroyed.....                                                        | Very coarse...                                               | 50                      | 5.850<br>65            | 3.920<br>2.370          | 5.1<br>10               | 3.8<br>7.4                  |                            |
| 60           | 26 Untreated<br>7% NaOH. | 25                         | 1 minute...           | 5 minutes in sul-<br>phuric acid of<br>10 per cent.<br>strength at 15°<br>C., washed with<br>cold water and<br>dried.                                  | Retained.....                                                         | Very soft elas-<br>tic and re-<br>sembling real<br>silk.     | 55                      | 4.918<br>68            | 3.072<br>4.710          | 6.5<br>9.4              | 4.5<br>4.1                  |                            |
| 65           | 27 Untreated<br>7% NaOH. | 15                         | 1 minute...           | 5 minutes in sul-<br>phuric acid of<br>10 per cent.<br>strength at 15°<br>C., 1 minute in<br>boiling water,<br>washed with<br>cold water and<br>dried. | Destroyed.....                                                        | Stiff, hard,<br>coarse, fila-<br>ments pas-<br>ted together. | 75                      | 5.053<br>94            | 3.086<br>2.920          | 5.4<br>8.6              | 4.1<br>5.3                  |                            |
| 70           | 28 Untreated<br>7% NaOH. | 25                         | 1 minute...           | 5 minutes in sul-<br>phuric acid of 10<br>percent strength<br>at 15° C., 1 min-<br>ute in boiling<br>water, washed<br>with cold water<br>and dried.    | Retained.....                                                         | Soft.....                                                    | 48                      | 5.725<br>60            | 4.604<br>4.360          | 6<br>11.6               | 4<br>6.3                    |                            |
| 75           | 29 Untreated<br>8% NaOH. | 15                         | 1 minute...           | 5 minutes in sul-<br>phuric acid of 10<br>percent strength<br>at 15° C., finally<br>washed and<br>dried.                                               | Completely<br>destroyed.                                              | Filaments are<br>pasted to-<br>gether.                       | 69                      | 5.043                  | 3.202                   | 6.2                     | 4.2                         |                            |

75

| Ex-<br>ample | Shrinking<br>agent                     | Tem-<br>pera-<br>ture      | Duration<br>of action | After-treatment                                                                                          | Lustre                    | Feel                      | Titre               | Strength per<br>dexter  |                         | Extens-<br>ibility         | Elast-<br>icity            | 5  |
|--------------|----------------------------------------|----------------------------|-----------------------|----------------------------------------------------------------------------------------------------------|---------------------------|---------------------------|---------------------|-------------------------|-------------------------|----------------------------|----------------------------|----|
|              |                                        |                            |                       |                                                                                                          |                           |                           |                     | In dry<br>state         | In wet<br>state         |                            |                            |    |
| 5            |                                        | Degrees<br>centi-<br>grade |                       |                                                                                                          |                           |                           |                     |                         |                         |                            |                            |    |
| 10           | 30 Untreated<br>8% NaOH                | 100                        | 1 minute              | 5 minutes in sul-<br>phuric acid of 10<br>percent strength<br>at 15° C.; finally<br>washed and<br>dried. | Completely<br>retained.   | Soft and elas-<br>tic.    | Deniers<br>66<br>69 | Grams<br>4.742<br>4.804 | Grams<br>3.460<br>3.347 | Per-<br>cent<br>4.4<br>7.8 | Per-<br>cent<br>3.1<br>4.5 | 10 |
| 15           | 31 Untreated<br>10% NaOH               | 15                         | 1 minute              | 5 minutes in sul-<br>phuric acid of 10<br>percent strength<br>at 15° C.; finally<br>washed and<br>dried. | Completely<br>destroyed.  | Somewhat soft.            | 62<br>78            | 4.435<br>1.625          | 2.758<br>0.746          | 5.7<br>12.2                | 4.4<br>5.6                 | 15 |
| 20           | 32 Untreated<br>10% NaOH               | 100                        | 1 minute              | 5 minutes in sul-<br>phuric acid of 10<br>percent strength<br>at 15° C.; finally<br>washed and<br>dried. | Completely<br>retained.   | Very soft and<br>elastic. | 53<br>56            | 4.603<br>3.901          | 2.320<br>2.062          | 5.4<br>8.4                 | 4.1<br>4.4                 | 20 |
| 25           | 33 Untreated<br>12% NaOH               | 15                         | 1 minute              | 5 minutes in sul-<br>phuric acid of 10<br>percent strength<br>at 15° C.; finally<br>washed and<br>dried. | Completely<br>destroyed.  | Somewhat soft.            | 65<br>90            | 4.861<br>1.475          | 3.276<br>0.813          | 6.3<br>10                  | 4.3<br>4.2                 | 25 |
| 30           | 34 Untreated<br>12% NaOH               | 100                        | 1 minute              | 5 minutes in sul-<br>phuric acid of 10<br>percent strength<br>at 15° C.; finally<br>washed and<br>dried. | Retained.                 | Soft and elastic.         | 53<br>59            | 4.490<br>3.923          | 2.528<br>2.389          | 5.6<br>9.4                 | 4.3<br>4.8                 | 30 |
| 35           | 35 Untreated<br>15% NaOH               | 15                         | 1 minute              | 5 minutes in sul-<br>phuric acid of 10<br>percent strength<br>at 15° C.; finally<br>washed and<br>dried. | Slightly de-<br>creased.  | Soft.                     | 67<br>86            | 5.164<br>2.502          | 3.529<br>1.700          | 5.7<br>10.7                | 4.4<br>4.1                 | 35 |
| 40           | 36 Untreated<br>15% NaOH               | 100                        | 1 minute              | 5 minutes in sul-<br>phuric acid of 10<br>percent strength<br>at 15° C.; finally<br>washed and<br>dried. | Completely re-<br>tained. | Very soft and<br>elastic. | 68<br>75            | 5.676<br>5.046          | 4.007<br>3.480          | 4.3<br>8.4                 | 3<br>4.4                   | 40 |
| 45           | 37 Untreated<br>20% NaOH               | 15                         | 1 minute              | 5 minutes in sul-<br>phuric acid of 10<br>percent strength<br>at 15° C.; finally<br>washed and<br>dried. | Slightly de-<br>creased.  | Soft.                     | 68<br>82            | 4.816<br>3.737          | 3.213<br>2.445          | 6<br>13.3                  | 4.7<br>4                   | 45 |
| 50           | 38 Untreated<br>20% NaOH               | 100                        | 1 minute              | 5 minutes in sul-<br>phuric acid of 10<br>percent strength<br>at 15° C.; finally<br>washed and<br>dried. | Completely re-<br>tained. | Soft and elastic.         | 53<br>60            | 4.669<br>4.000          | 2.783<br>2.525          | 5<br>9                     | 3.7<br>4.4                 | 50 |
| 55           | 39 Untreated<br>74% NaOH               | 150                        | 1 minute              | 5 minutes in sul-<br>phuric acid of 10<br>percent strength<br>at 15° C.; finally<br>washed and<br>dried. | Completely re-<br>tained. | Soft and elastic.         | 73<br>76            | 4.589<br>4.296          | 2.808<br>2.730          | 6<br>8.5                   | 4<br>4.5                   | 55 |
| 60           | 40 Untreated<br>58% Na <sub>2</sub> S  | 15                         | 5 minutes             | 5 minutes in sul-<br>phuric acid of 10<br>percent strength<br>at 15° C.; finally<br>washed and<br>dried. | Slightly de-<br>creased.  | Soft.                     | 54<br>62            | 4.416<br>3.217          | 2.500<br>1.822          | 5.5<br>9.7                 | 4.2<br>5.1                 | 55 |
| 65           | 41 Untreated<br>58% Na <sub>2</sub> S  | 100                        | 5 minutes             | 5 minutes in sul-<br>phuric acid of 10<br>percent strength<br>at 15° C.; finally<br>washed and<br>dried. | Completely re-<br>tained. | Soft and elas-<br>tic.    | 68<br>71            | 5.242<br>5.281          | 3.691<br>3.661          | 4.6<br>7.1                 | 3.3<br>5.1                 | 60 |
| 70           | 42 Untreated<br>84% Na <sub>2</sub> S  | 50                         | 5 minutes             | 5 minutes in sul-<br>phuric acid of 10<br>percent strength<br>at 15° C.; finally<br>washed and<br>dried. | Completely re-<br>tained. | Soft and elas-<br>tic.    | 74<br>74            | 4.797<br>5.074          | 3.412<br>3.702          | 4.4<br>7.5                 | 3.1<br>4.9                 | 65 |
| 70           | 43 Untreated<br>100% Na <sub>2</sub> S | 100                        | 5 minutes             | 5 minutes in sul-<br>phuric acid of 10<br>percent strength<br>at 15° C.; finally<br>washed and<br>dried. | Completely re-<br>tained. | Soft and elas-<br>tic.    | 53<br>53            | 4.811<br>4.470          | 2.594<br>2.960          | 5.5<br>8                   | 4.2<br>4.7                 | 70 |

From the foregoing tables the following facts are evident:—

A solution of caustic soda of 7 per cent. strength at room temperature completely destroys the lustre of ordinary viscose silk and Lillienfeld-silk. The same solution applied at 25° C. does not damage the lustre and does not considerably decrease the dry and wet tenacity; it increases the extensibility and elasticity to a great extent.

10 In the present process there may be used as treating baths, caustic alkali solution of any strength from 3 per cent. (calculated as NaOH) up to solutions saturated at the temperature desired for the treatment, and alkali metal sulphide 15 solutions of any strength from 15 per cent. (calculated as crystalline sodium sulphide,  $Na_2S \cdot 9H_2O$ ) up to solutions saturated at the temperature desired for the treatment. And temperatures of from 25 to 160° C. may be employed—  
20 provided that when very high temperatures, for example temperatures exceeding 100° C. are used, the time of treatment is accordingly shortened.

Consequently, in the foregoing examples there may be used any temperature between 25 and 160° C., for example 40° C., or 50° C., or 70° C. etc.

A solution of caustic soda of 8 per cent. strength at room temperature completely destroys the lustre of ordinary viscose silk and of Lillienfeld-silk, and causes the silk to swell or dissolve to such an extent that the fibres are caused to adhere to each other. The same solution applied at 100° C. does not damage the lustre; it decreases the strength in wet and dry condition in the case of ordinary viscose silk only inappreciably and in the case of Lillienfeld-silk not at all; it increases the extensibility of both kinds of silk very considerably and it scarcely affects the elasticity of the ordinary silk and increases that of Lillienfeld-silk very considerably.

40 A solution of caustic soda of 10 per cent. strength at ordinary room temperature destroys the lustre of ordinary viscose silk and of Lillienfeld-silk, and causes an extraordinary decrease in the strength of both kinds of silk in the wet and dry state, so that the increase in extensibility also produced is without value. The same solution applied at 100° C. causes no appreciable diminution in the lustre of either kind of silk, decreases only inappreciably the strengths in the wet and dry state, and causes a considerable increase in the extensibility and elasticity.

45 A solution of caustic soda of 12 per cent. strength, at ordinary room temperature destroys the lustre of both kinds of silk and causes a great reduction in the strength in wet and dry state, and moreover, greatly diminishes the elasticity of ordinary viscose silk; all these disadvantages outweigh the value of the increased extensibility produced by the treatment. The same solution applied at 100° C. does not reduce the lustre of either kind of silk, reduces only slightly the strength in the wet and dry state, and increases considerably the extensibility and elasticity.

50 A solution of caustic soda of 15 per cent. strength at 15° C. reduces the lustre and causes, in the case of both kinds of silk, a considerable decrease in the strength in the wet and dry state and in the elasticity; the increase in extensibility simultaneously produced is therefore of no value. 55 When the same solution is applied at 100° C., the lustre is retained, the strength in the wet and dry state suffers an inappreciable diminution, and the elasticity and extensibility are appreciably increased.

75 A solution of caustic soda of 18 per cent.

strength at 15° C. reduces considerably the lustre and the strength in the wet and dry state of ordinary viscose silk, and has no appreciable effect on its elasticity; the increase in extensibility is, therefore, of no importance. When the same solution is applied at 100° C. the lustre is preserved, the strength in wet and dry state is slightly diminished, the extensibility is increased considerably and the elasticity very considerably.

80 A solution of caustic soda of 20 per cent. strength used at ordinary room temperature reduces the lustre of ordinary viscose silk and slightly reduces that of Lillienfeld-silk; in the case of ordinary viscose silk the strength in the wet and dry state is considerably decreased, and in the case of Lillienfeld-silk is decreased, but less considerably; the extensibility of both kinds of silk is improved, but their elasticity is very considerably diminished. When the same solution is applied at 100° C. the lustre of both silks is unaffected, the decrease in their strengths in wet and dry state is very slight and the extensibility and elasticity increase, the latter by about 100 per cent. in the case of viscose silk.

85 A solution of caustic soda of 22.5 per cent. strength at ordinary room temperature detracts from the lustre of ordinary viscose-silk and causes a considerable decrease in its strength in wet and dry state, an increase in its extensibility and a decrease in its elasticity. The same solution applied at 120° C. does not decrease the lustre, decreases the strength but slightly, and increases the extensibility and elasticity.

90 A solution of crystallized sodium sulphide of 58 per cent. strength at ordinary room temperature reduces the lustre of both kinds of silk, so that the increase in extensibility and elasticity are rendered valueless. When the same solution is used at 100° C., both kinds of silk retain their original lustre, hardly suffer in respect of their strength, in the wet and dry state, and acquire a considerable increase in their extensibility and elasticity.

95 By treating an artificial silk fabric from ordinary viscose silk with a hot or warm solution of an alkali or alkali sulphide, in a manner similar to that described in the preceding examples, for instance, the following results are obtained:—

A solution of caustic soda of 5 per cent. strength at 15° C. causes a strong diminution in the lustre and renders the material stiff and coarse to the feel. If the same solution is used at 100° C., the lustre is preserved and the material acquires a completely silky character, and a soft feel.

100 A caustic soda solution of 7 per cent. strength at 15° C. diminishes the lustre and makes the feel of the material very stiff. The same solution employed at 25° C., does not affect the lustre and imparts to the fabric a soft feel.

105 A solution of caustic soda of 20 per cent. strength at ordinary temperature practically destroys the lustre and confers on the material a stiff, coarse feel. If the same solution is used at 100° C., the metallic lustre gives place to a wholly silky appearance and the material becomes very soft to the feel.

110 When using a solution of caustic soda of 50 per cent. strength at 50° C., the lustre is practically the same as that of natural silk, and the material acquires a very soft feel. If the same solution is applied at 100–140° C., the material acquires a lustre which cannot be distinguished from that of natural silk, and its feel becomes soft and crackling.

115 Even caustic soda solutions of 74 per cent.

strength used at 150° C. give to fabrics consisting of ordinary viscose silk properties which are similar to those of natural silk.

Solutions of sodium sulphide of 58, 84 and 100 5 per cent. strength (calculated as crystalline  $\text{Na}_2\text{S}$ ) at 100-150° C. also confer upon fabrics of artificial silk a lustre which approaches or is even equal to that of natural silk, and a very soft feel.

A very important result of the treatment of 10 artificial fibrous material with a warm or hot solution of an alkali or of an alkali sulphide, as described in the foregoing examples, is that the tendency of the material to form creases which do not disappear is very much diminished or even 15 eliminated.

The treatment described in the foregoing examples may be applied to artificial fibrous material whilst this is subjected to tension, but the effects of the treatment, whilst they are still appreciable are less pronounced than when no tension is applied.

The treatment of spun or woven mixed materials containing artificial fibrous material, as well as the treatment of staple fibre, will be understood from the foregoing examples.

In the foregoing examples, instead of the temperatures given therein for the caustic soda solutions or sodium sulphide solutions, there may be used other temperatures, for example, any 30 temperatures between 25 and 100° C.

In the foregoing examples, there may be used, instead of the solutions therein prescribed, a solution of another basic substance, for example, a solution of guanidine of 20-50 per cent. strength, 35 the temperature of the treatment being, for example, 25-100° C.; so also instead of a solution of caustic soda, there may be used a solution of another caustic alkali, such as a caustic potash solution of equivalent strength; and instead of 40 a solution of sodium sulphide a solution of another alkali metal sulphide may be used, such as potassium sulphide. There may also be used a strong solution of trimethyl-sulphonium hydroxide, of tetramethyl-ammonium hydroxide or the 45 like.

The treatment of artificial silk other than viscose silk, for example cuprammonium silk, is conducted in a similar manner, but it may be mentioned that in the case of the treatment of 50 cellulose acetate silk, the solution of the basic substance should be concentrated; for example, a caustic soda solution of 36 per cent. strength used at 100° C. or of 50 per cent. strength used at 100-140° C. is suitable.

55 Instead of transferring the artificial fibrous material directly from the hot alkali solution to an acid bath, as described in the examples, it may be introduced into cold or warm or boiling water after being removed from the hot alkali solution 60 (see, for instance, Examples 21, 22, 27 and 28), and then washed, if required after being treated with an acid, and finally dried.

I claim:

1. A process for treating artificial fibrous material of regenerated cellulose, which comprises acting on said material with a solution selected 65 from the herein described group consisting of

caustic alkali solution of not less than 3% strength, calculated as  $\text{NaOH}$ , and alkali metal sulphide solution of not less than 15% strength, calculated as  $\text{Na}_2\text{S}\cdot 9\text{H}_2\text{O}$ , and at a temperature not less than 50° C., thereafter washing and drying said material.

2. A process for treating artificial fibrous material, which comprises acting on said material with a solution of an alkali sulphide containing not less than 50 per cent. alkali sulphide (calculated as crystalline sodium sulphide) at a temperature of not less than 50° C.

3. A process for treating artificial fibrous material produced by spinning viscose into a coagulating bath containing not less than 50 per cent. 15 of  $\text{H}_2\text{SO}_4$ , which comprises acting on said material with an alkaline solution selected from the herein described group consisting of caustic alkali solution of at least 5% concentration, calculated as  $\text{NaOH}$ , and alkali metal sulphide solution of at 20 least 15% concentration, calculated as  $\text{Na}_2\text{S}\cdot 9\text{H}_2\text{O}$ , which solution has a temperature not less than 50° C., thereafter washing and drying said material.

4. A process as in claim 3, wherein a caustic 25 soda solution is used as the alkaline solution.

5. A process as in claim 3, wherein the artificial fibrous material after being treated with the alkaline solution is contacted with an acid solution and then washed and dried.

6. A process for treating artificial fibrous material produced by spinning viscose into a coagulating bath containing not less than 50 per cent. of 35  $\text{H}_2\text{SO}_4$ , which comprises acting on said material with a solution of an alkali sulphide containing not less than 15 per cent. of alkali sulphide (calculated as crystalline  $\text{Na}_2\text{S}$ ) at a temperature of not less than 50° C.

7. A process as in claim 6, wherein the strength of the sodium sulphide solution (calculated as 40 crystalline  $\text{Na}_2\text{S}$ ) is not less than 50 per cent.

8. A process for treating artificial fibrous material produced by spinning viscose into a coagulating bath containing not less than 50 per cent. of  $\text{H}_2\text{SO}_4$ , which comprises acting upon said material with a solution consisting of melted crystalline sodium sulphide at about 100° C., thereafter washing and drying the material.

9. A process of improving cellulose acetate threads which comprises subjecting said threads to the action of a treating solution selected from the group consisting of (a) caustic alkali solution of not substantially below 30% strength, calculated as  $\text{NaOH}$ , and (b) alkali metal sulphide solution of about 84 to 100%, calculated as  $\text{Na}_2\text{S}\cdot 9\text{H}_2\text{O}$ ; 55 such treatment being effected at a temperature not substantially below 50° C., and thereafter washing and drying the said threads.

10. A process as set forth in claim 3 in which a caustic alkali solution is used and in which the 60 time of treatment does not exceed five minutes.

11. A process as set forth in claim 3 in which a caustic alkali solution is used having a strength of not less than 3 per cent (calculated as  $\text{NaOH}$ ), and in which the time of treatment does not exceed 65 five minutes.

LEON LILIENFELD.